

Aug. 28, 1945.

J. C. F. C. RICHTER

**2,383,684**

## PROCESS OF CONTINUOUS ALKALI TREATMENT OF FIBROUS MATERIAL

Filed April 29, 1942

3 Sheets-Sheet 1



Inventor:  
Johan Christoffer Fredrik Carl Richter

By George Bayard Jones  
Attorney

Aug. 28, 1945.

J. C. F. C. RICHTER

2,383,684

## PROCESS OF CONTINUOUS ALKALI TREATMENT OF FIBROUS MATERIAL

Filed April 29, 1942

3 Sheets-Sheet 2



Fig. 2.

### Inventori:

Johan Christoffer Fredrik Carl Richter  
By George Bayard Jones  
Attorney

Aug. 28, 1945.

J. C. F. C. RICHTER

2,383,684

PROCESS OF CONTINUOUS ALKALI TREATMENT OF FIBROUS MATERIAL

Filed April 29, 1942

3 Sheets-Sheet 3



Inventor:

Johan Christoffer Fredrik Carl Richter  
By George Bayard Jones  
Attorney

## UNITED STATES PATENT OFFICE

2,383,684

## PROCESS OF CONTINUOUS ALKALI TREATMENT OF FIBROUS MATERIAL

Johan Christoffer Fredrik Carl Richter, Oslo,  
Norway, assignor to Aktiebolaget Kamyr,  
Karlstad, Sweden, a company of Sweden

Application April 29, 1942, Serial No. 446,966  
In Sweden November 8, 1940

2 Claims. (Cl. 92—13)

This invention relates to a process of continuous alkali treatment of fibrous material, i. e., material consisting of fibers, such as cellulose fibers produced by digestion of fiber-containing raw materials. The fibrous material to be treated may or may not have been previously subjected to chlorination and concentration.

The course of this alkali treatment process is determined, inter alia, by two factors, namely the strength of liquor and the temperature used. The higher consistency that the fiber pulp possesses, that is to say, the less water it contains, the less quantity of alkali is obviously required to obtain a certain desired strength of the liquor, and the less heat is required to attain the required temperature. But in practice the possibility of utilizing a high consistency of the fiber pulp is limited by the necessity of effecting an efficient mixture of the fiber pulp or material and the liquor, and also by the difficulty of effecting conveyance of fiber material possessing a high consistency through the apparatus used and the discharge of such material from the apparatus after the treatment has been finished. In view of these factors a consistency of between 15 and 18 percent of the mixture of fiber material and liquor has hitherto been regarded as the highest consistency possible in actual practice. At the said consistency of from 15 to 18 per cent it is possible to feed the mixture or pulp into and discharge the same from the tower or tank in which the alkali treatment is carried out, but to attain the said consistency it is necessary to overcome certain difficulties. It will be obvious that for obtaining the said consistency of 15 to 18 per cent of the mixture of fiber material and liquor, the material supplied to the mixing apparatus must previously have been concentrated to a higher consistency, for instance 20 to 25 per cent.

This necessitates the use of grooved presses or other apparatus suitable for the purpose, which obviously increases the cost of the plant as well as of the operation. At the consistency mentioned difficulties are also met with in attaining an efficient mixture of the fiber material and the liquor, since, in order not to dilute the pulp more than absolutely necessary, the liquor must be added in a concentrated state, that is to say, in small quantities, and it is of course very difficult to obtain a uniform distribution of these small quantities in the concentrated mass of material, particularly in view of the fact that the material will easily roll into balls during the mixing operation instead of breaking up and becoming dispersed in the liquor.

These difficulties and inconveniences are eliminated in a simple and efficient manner according to the present invention. The process according to the invention consists principally in intimately mixing the fiber material in a suitable mixing apparatus with so large a surplus quantity of alkali liquor of a strength required for the treatment that a uniform distribution of the alkali in the material is effected, and so that the mixture of material and liquor obtains such consistency that it can afterwards be conveyed to a reaction chamber as a flowing liquid. Before or simultaneously with the introduction of the material into the reaction chamber, so large a quantity of liquor is separated from the mixture or pulp that the material entering the reaction chamber possesses the desired concentration which is suitable for the reaction to take place in said chamber. The separation of surplus liquor from the mixture to obtain the desired concentration of the material before the introduction of the same into the reaction chamber, may preferably be carried out by pressure, and such pressure may be suitably be utilized also to effect the introduction of the material into the reaction tank and to feed said material into and convey it through said tank.

According to this invention, therefore, the operation is carried out with a surplus quantity of liquor with a view to secure a uniform mixture and impregnation of the material with liquor, and also to facilitate an easy and continuous conveyance of the mixture to the reaction tank. This surplus quantity of alkali liquor is recovered in connection with the introduction of the material into the reaction tank, for instance by subjecting the mixture to a pressing operation, and such surplus quantity may thus be re-used for diluting further quantities of material and may thus circulate through the system.

When the process is carried out with the use of a circulating quantity of liquor, a portion of said circulating liquor may be used, according to a further embodiment of the invention, for the purpose of removing by displacement some of the water contained in the fiber material to be treated before such material is supplied to the mixing apparatus, the remaining portion of the circulating liquor being supplied as a diluting liquid to the mixing apparatus for the purpose of producing the desired uniform distribution of the alkali liquor in the fiber material and a suitable consistency of the mixture for enabling it to be conveyed as a flowing liquid to the reaction tank. In order to secure the desired concentra-

tion of the material suitable for the treatment of the same in the reaction chamber, the mixture is also in this case relieved of the surplus quantity of liquor before or in connection with the introduction of the material into the reaction chamber. The quantity of liquor thus removed from the material corresponds substantially to the quantities used for the displacement operation and for the dilution of the material in the mixing apparatus, and is returned as circulating liquor to be re-used for the same purposes.

By utilizing in this manner a portion of the circulating liquor for displacement of some of the water contained in the material supplied to the process, the necessity is avoided of using grooved presses or the like for removing the water, and the problem of supplying the material with the least possible content of water is thus solved in a simple and efficient manner. The liquor used for the displacement operation remains in the fiber material and is conveyed with the latter to the mixing apparatus where it cooperates with the portion of the circulating liquor which is supplied as a diluting liquid to the mixing apparatus, to effect a uniform and efficient mixing and impregnation of the material and to produce a mixture of a consistency suitable for an easy conveyance through the apparatus.

For a more complete understanding of the present invention a few constructional forms of apparatus suitable for performing the present process are illustrated in the accompanying drawings by example and somewhat diagrammatically, i. e. in the form of flow sheets. Fig. 1 illustrates an apparatus in which the material is introduced at the lower end of the reaction chamber. Fig. 2 shows a similar apparatus which includes means for removal of water by displacement from the fiber material to be treated. Fig. 3 illustrates an apparatus in which the material is introduced at the top of the reaction chamber, and Fig. 4 shows a modified apparatus of the same type. The various apparatus illustrated in the drawings may, for instance, constitute the second step of a bleaching plant in the first step of which the material is chlorinated, after which the material is subjected to treatment with alkali in the second step.

Referring to Fig. 1, the fiber material which thus may be chlorinated, is first supplied to a filter apparatus 1 having grooved pressure rolls in which it may be thickened to a consistency of, for instance, 20 to 22 per cent, which may be raised to 25 to 28 per cent by afterwards passing the stock through a grooved press, not shown in the drawings.

The stock is then passed to the apparatus for the alkali treatment which mainly consists of a mixing apparatus 2 and a reaction tank 3 which are connected to one another by means of a pipe or conduit 4. Located above the mixer 2 is a receptacle 5 from which strong alkali liquor is conducted through a conduit 7 provided with quantity adjusting means 6 to a conduit 8 which serves for the supply of circulating liquor, and through said conduit 8 to the mixer 2. The quantity of circulating liquor supplied is such that due to the mixing operation in the mixer 2 the pulp obtains a consistency of about 5 to 8 per cent. Due to this considerable dilution the alkali liquor is intimately and uniformly mixed with the fibrous material, and the mixture obtains at the same time a sufficiently liquid consistency to render it possible to convey the same as a flowing liquid through pipes and bends.

The pipe or conduit 4 leading from the mixer 2 is connected to an angle pipe 9, and between said pipe 9 and the lower or entrance end or opening of the reaction tank 3 a sieve chamber 10 is provided from which a discharge pipe 11 provided with a regulating valve 12 leads to a collecting receptacle 13. In said sieve chamber 10 the liquor is separated to the desired extent from the material continuously conveyed downwards through the pipe 4 to the angle pipe 9. The liquor is pressed out from the material and the continued feeding of the latter through the reaction tank 3 is effected by a press and conveyer worm 14 or the like which is located within the sieve chamber 10 and which is driven from the outside by means of any suitable device, which is indicated at 15. By means of the press and conveyer worm 14 such quantity of liquor is expressed from the material that the latter obtains a consistency of about 20 to 25 per cent.

The removal of the expressed alkali liquor is effected under control of the regulating valve 12 which is regulated by the level of the liquor in the receptacle 13 by any suitable means diagrammatically illustrated in the drawings as a float and lever arrangement generally referenced 25. The arrangement is such that the valve 12 decreases the area of flow through the conduit 11 when the liquor rises in the collecting receptacle 13, and increases said area of flow when the level of liquor in said receptacle falls. A pump 17 conveys the expressed surplus quantity of liquor from the collecting receptacle 13 through a conduit 16, and if desired through a calorizer 18, to the above-mentioned conduit 8 and back to the mixer 2. Heating of the material may also be effected during the mixing by supplying steam into the mixer 2 through the steam conduit 24.

In the unit of time a constant quantity of pulp 40 having a constant percentage of dry matter is supplied from the filter apparatus 1 to the mixer 2. Likewise, the quantity of fresh liquor supplied from the receptacle 5 to the mixing apparatus 2 in the unit of time is constant, and if heating is 45 effected by supply of direct steam through the steam pipe 24, the quantity of steam supplied in the unit of time is also constant. By means of the valve 20 in the conduit 16 the quantity of circulating liquor supplied by the pump 17 through said conduit 16 is adjusted in such manner that the desired suitable consistency of the pulp in the mixing apparatus 2 is obtained. Since the valve 12 controls the discharge of expressed liquor from the lower end of the tank 3 in such manner that the level of liquor in the receptacle 13 is maintained constant, or in other words, in such manner that the discharged quantity of expressed liquor corresponds exactly to the quantity of liquor conveyed by the pump 17, it will be understood 55 that a constant quantity of liquor which is dependent upon the adjustment of the valve 20, will circulate through the system.

As a result hereof the material or pulp charged into the reaction tank 3 by the press and conveyer worm 14 will also possess a constant consistency which in this case corresponds to the constant quantities of pulp, fresh liquor, and steam supplied to the mixing apparatus 2.

If liquor is required at some other point in 70 the plant, however, for instance for neutralizing after the pretreatment of the material with chlorine, a portion of the liquor may be withdrawn from the system, for instance at 19. This withdrawal of liquor should be effected continuously, 75 so that a constant quantity of liquor is withdrawn

in the unit of time. In this case the quantity of expressed liquor discharged from the lower end of the reaction tank through the valve 12 will correspond to the sum of the circulating quantity of liquor, the quantity of which is adjusted by means of the valve 20, and the quantity of liquor withdrawn at 19. Since these two quantities of liquor are constant, the pulp charged into the reaction tank 3 will also in this case have a constant consistency, which corresponds to the difference between the sum of the quantities of pulp, fresh liquor, and steam supplied to the mixing apparatus 2, and the quantity of liquor withdrawn at 19.

The liquor circulated by the pump 17 may also be allowed first to pass through an evaporation apparatus before it is supplied to the mixing apparatus 2, for in this manner to increase the liquor concentration of the pulp mixture, whereby the consumption of chemicals is reduced. If the evaporation is carried out in such manner that the quantity of water evaporated from the liquor in the unit of time is constant, a constant consistency of the pulp charged into the reaction tank 3 will also in this case be maintained, as will be easily understood.

The material charged into the reaction tank has a consistency of about 20 to 25 per cent and moves continuously upwards through the tank, until at the top thereof it is scraped over the rim 22 by a scraper 21 or the like which may be driven in any suitable manner, after which the material passes to a washing device 23. If desired, the material may afterwards be subjected to treatment with hypochlorite, for instance in a third step of the system.

The apparatus illustrated in Fig. 2 is largely arranged in the same manner as that above described in connection with Fig. 1, and like reference numerals are used to designate the same parts. The material to be treated, which also in this case may or may not be previously chlorinated, is first supplied to a suitable apparatus, such as a filter apparatus 31, by means of which a portion of the water contained in the material may be removed by displacement by means of circulating liquor which is supplied through the pipes 56. The advantage of such displacement of the water will easily be understood from the following consideration. With a filter apparatus it is possible to thicken the supplied pulp mixture to such extent that the pulp leaving the filter contains 12 per cent fiber or dry substance and 88 per cent water. By a displacement operation it is possible from this water content of 88 per cent to force out a quantity of water corresponding to 50 per cent, and to replace this quantity with displacement liquor, so that, not taking into account the water in the added liquor, the pulp leaving the filter contains 38 per cent water only. The pulp leaving the filter thus contains a percentage of fiber or dried matter which, figured on the total quantity of fiber and water but disregarding the added liquor, amounts to 24 per cent.

In this manner, merely by displacement and with the use of a simple apparatus, substantially the same reduction is obtained of the water content in the pulp which shall afterwards be supplied to the mixing apparatus, for obtaining which it was hitherto necessary to use grooved presses or other expensive and power-consuming apparatus.

When the pulp has been concentrated in this manner relatively to the quantity of water remaining in the same, it is conveyed from the filter

apparatus 31 to the apparatus for the alkali treatment, which, as already stated, is arranged in substantially the same manner as that above described with reference to Fig. 1. The pulp first enters the mixing apparatus 2 to which strong alkali liquor is supplied from the receptacle 5 through the pipe 7 provided with a regulating valve 6, while circulating liquor is supplied to the mixer 2 through the pipe 8 provided with a valve 10. The supply of circulating liquor through the pipes 56 for the displacement operation on the filter apparatus 31, and through the pipe 8 to the mixer 2, is adjusted by means of the valves 57 and 20 in such manner that due to the mixing in said mixer 2 the pulp obtains a suitable consistency, for instance 5 to 8 per cent, so that the alkali liquor is intimately and uniformly mixed with the fibrous material, and the consistency is sufficiently liquid to enable the mixture to be conveyed as a flowing liquid through pipes and conduits. The mixer 2 is connected through the downflow pipe 4 with the angle pipe 9 which is connected over the sieve chamber 10 with the inlet end of the reaction tank 3. In the sieve chamber 10 liquor is expressed from the material to the desired extent by means of the rotatable press or conveyor worm 14 which is driven by suitable means indicated at 18.

The worm 14 also serves to feed the material continuously upward in the tank 3 until at the top of the latter the scraper 21 scrapes the material over the rim 22 after which the material is conveyed to the washing device 23. By means of the worm the material is pressed to a consistency of about 20 to 25 per cent. The expressed liquor is conveyed from the sieve chamber 10 to the tank 13 through the pipe 11 which is provided with the regulating valve 12 which is controlled by the level of liquor in the tank 13 by the float and lever arrangement 25 in such manner that the flow through the valve is decreased when the level rises in the tank 13 and is increased when the level in the tank falls. The liquor discharged in the tank 13 is conveyed by the pump 17 through a conduit 16, and if desired, through a calorizer 18, to the abovementioned pipe 8 and through the regulating valve 57 to the pipes 56 to be used again for dilution in the mixer 2 and for displacement on the filter 1. Also in this case a steam conduit 24 is provided for effecting heating of the material, if desired, by introducing steam into the mixer 2.

Also in this case the filter 31 shall operate in such manner that in the unit of time it delivers a constant quantity of pulp having a constant content of fiber or dry matter. Likewise, the quantity of fresh liquor supplied from the receptacle 5 to the mixer 2 in the unit of time is constant, and if heating is effected by means of steam supplied through the pipe 24, the quantity of steam supplied in the unit of time shall also be constant. By means of the valves 57 and 20 the quantity of circulating liquor supplied by the pump 17 through the conduit 16 is adjusted in such manner that the desired displacement is obtained on the filter 1 and the desired suitable consistency of the pulp is obtained in the mixer 2.

Since the valve 12 controls the discharge of expressed liquor from the lower end of the reaction tank 3 in such manner that the level of liquor in the tank 13 is maintained constant, and consequently, the quantity of expressed liquor discharged to the tank corresponds exactly to the quantity of liquor conveyed by the pump 17, it will be understood that a constant quantity of

liquor will circulate through the system, and that this quantity is dependent upon the adjustment of the valves 57 and 20. Accordingly, the material fed into the reaction tank 3 by the press and conveyer worm 14 will also possess a constant consistency which in this case corresponds to the sum of the constant quantities of dry matter and water—with the exception of the displacement liquor—contained in the pulp supplied to the mixer 2 and the constant quantities of fresh liquor and steam. If it is desired that the pulp material charged into the tank 13 shall have a consistency higher than that which corresponds to the sum of the said constant quantities, a quantity of liquor constant in the unit of time may be withdrawn, for instance through the branch pipe 19 on the conduit 18, in which case the pulp charged into the reaction tank 3 obtains a constant consistency which corresponds to the difference between the abovementioned constant quantities supplied to the mixing apparatus 2 and the quantity of liquor drained off at 19.

In the constructional form illustrated in Fig. 3 a plurality of the parts illustrated in Fig. 2 are used and are designated by like reference numerals. The constructional form illustrated in Fig. 3 differs from that illustrated in Fig. 2 principally in that the sieve chamber 10 containing the press and conveyer worm 14 is not connected to the lower end of the reaction tank, but is located above the reaction tank 63.

The material which has been subjected to pressure in the press and conveyer device 10, 14, falls from the outlet 79 of said device into the reaction tank 63, which in this case consists of a tower in which the material gradually sinks downward and from the lower end of which it is discharged by the aid of a stirrer 81. Also in this case the discharge of the expressed liquor from the sieve chamber 10 through the discharge pipe 11 is controlled by the valve 12 in said pipe which in its turn is controlled by the level of the liquor in the tank 13 through the device 25, so that in this manner a constant quantity of liquor always circulates through the system, and consequently, the material delivered to the tower 63 always has a constant consistency.

Also in the constructional form illustrated in Fig. 4 a plurality of the parts previously described are used, and they are designated by the same reference numerals. This constructional form differs from that described in connection with Fig. 3 in that the pulp mixture discharged from the mixer 2 flows through the pipe 4 to a thickener or uptaking machine 90 in which the liquor is removed and expressed from the fibrous material to the required extent, after which the material may be allowed to pass through a shredder 91 and then falls into the tower 63. Also in this case the discharge conduit 11 for the expressed liquor from the uptaking machine 90 to the tank 13 is provided with a control valve 12 which is controlled by the level of liquor in said tank through the float and lever arrangement 25 in such manner that the function and the operation become the same as those above described.

For the purpose of mercerizing cellulose, for instance for the manufacture of artificial silk, an apparatus arranged in accordance with the principles above explained, may be used, with the sole modification that in such case the mixing apparatus 2 is combined with a reaction zone in which the material is subjected to alkali treatment during a few minutes, and that the tower will correspond to the ripening apparatus for the mercer-

ized material. In this case it is desired to obtain a concentration of about 30 per cent dry matter by means of the press device 14 or the uptaking machine 90. Consequently, it is desirable in this case to carry out the displacement operation on the filter 31 as far as possible, so as not to introduce an unnecessary quantity of water into the process.

The constructional forms above described and illustrated in the drawings are only to be regarded as examples, and it will be understood that they may be modified in several ways as regards their details without departing from the principle of the invention. In Figs. 1 and 2, for instance, the reaction tank may be located horizontally and may have a horizontal press and conveyer worm. In such case the material may be allowed to flow from the mixer straight down to the worm which expresses the excess liquor and feeds the pulp in the horizontal direction through the tank. At the other end of the tank the alkali-treated material may be allowed to drop over the edge of the tank without the aid of a mechanical discharge device, or it may be flushed over the edge. At the discharge end of the tank the material assumes in this case an angle of repose of about 45 degrees, and for this reason the tank should be made very narrow, that is, with a small diameter and a great length.

I claim:

1. The process of continuous alkali treatment of fibrous material, which consists in removing water from the fibrous material by displacement of water therein with alkali liquor, intimately mixing the fibrous material in a suitable mixing apparatus with a quantity of alkali liquor sufficient to effect treatment of said material and with an additional surplus quantity of alkali liquor sufficient to produce uniform distribution of the alkali in said material and a mixture of material and alkali liquor having a consistency such that said mixture is capable of being conveyed as a flowing liquid, causing such mixture of fiber material and liquor to flow to a reaction chamber, removing from said mixture preparatory to introducing it into said reaction chamber a quantity of alkali liquor substantially equal to the total quantity of alkali liquor used for displacement of water from the material and as surplus liquor mixed with the material in the mixing apparatus and such that due to its removal the material obtains a concentration suitable for the reaction, introducing said material into the reaction chamber, subjecting said material in said reaction chamber to treatment with the alkali liquor remaining in the material, employing a portion of such quantity of alkali liquor removed from the material preparatory to its introduction into the reaction chamber for removing water by displacement from a fresh quantity of fibrous material, and returning the remaining portion of such removed quantity of alkali liquor to the mixing apparatus and using such portion as surplus mixing liquor for a fresh quantity of fibrous material.

2. The process of continuous alkali treatment of fibrous material, which consists in removing water from the fibrous material by displacement of water therein with alkali liquor, intimately mixing the fibrous material in a mixing apparatus with a quantity of alkali liquor sufficient to effect treatment of said material and with an additional surplus quantity of alkali liquor sufficient to produce uniform distribution of the alkali in said material while providing a mixture of

material and alkali liquor having a consistency such that the mixture is capable of being conveyed as a flowing liquid, causing the mixture of fiber material and liquor to flow continuously to a reaction chamber, continuously subjecting said mixture to pressure so as to separate from the mixture a quantity of alkali liquor substantially equal to the total quantity of alkali liquor used for displacement of water from the material and as surplus liquor mixed with the material in the mixing apparatus thereby reducing the concentration of the mixture to a concentration suitable for the reaction, said pressure serving also to continuously introduce the mate-

rial into and convey the same through the reaction chamber, subjecting said material in said reaction chamber to treatment with the alkali liquor remaining in the material, employing a portion of the alkali liquor pressed out from the material for continuously removing water by displacement from fresh quantities of fibrous material, and continuously recycling the remaining portion of such pressed out alkali liquor to the mixing apparatus and using such portion as surplus mixing liquor for fresh quantities of fibrous material.

JOHAN CHRISTOFFER FREDRIK  
CARL RICHTER.